

# UNITED STATES PATENT OFFICE.

NIELS C. CHRISTENSEN, OF SALT LAKE CITY, UTAH, ASSIGNOR TO METALLURGIC IMPROVEMENT CORPORATION, OF SALT LAKE CITY, UTAH, A CORPORATION OF UTAH.

## PROCESS OF TREATING ORES BY FLOTATION.

1,286,531.

Specification of Letters Patent.

Patented Dec. 3, 1918.

No Drawing.

Application filed March 6, 1918. Serial No. 220,862.

To all whom it may concern:

Be it known that I, NIELS C. CHRISTENSEN, a citizen of the United States, residing at No. 637 E. 9 So., in Salt Lake City, in the 5 county of Salt Lake and State of Utah, have invented new and useful Improvements in the Processes of Treating Ores by Flotation, of which the following is a specification.

This invention relates to a process for the 10 treatment of copper ores and also ores containing copper and gold and silver. It is especially applicable to oxidized ores or ores which are partly oxidized. It is also applicable to sulfid ores which have been 15 given a preliminary roasting treatment. Although the invention has been found especially applicable to relatively low grade copper ores, it is also applicable to many ores which contain silver and gold as well as 20 copper.

The methods of applying my process are in some respects similar to the so-called flotation processes now so widely used, and may in part be carried out in the apparatus 25 now used in these processes; my process, however, depends upon an entirely new discovery. In my invention the valuable metal is separated by flotation, either by the frothing method now so widely used or by the film 30 tension method as used by Macquisten; but the invention differs from the old flotation processes in that the metal is not floated as a sulfid but as an entirely different compound which must first be made from the 35 minerals in the ore before treatment by flotation.

The compound of copper which possesses this property of "floating" to an even greater degree than the natural or artificially 40 prepared sulfids is the red cupro-cupric sulfite such as is formed by boiling off the  $\text{SO}_2$  from a solution of copper in water and  $\text{SO}_2$ , or such as is made by the action of  $\text{CuSO}_3$  in a dilute  $\text{SO}_2$  solution upon the oxidized 45 copper minerals, or by the action at proper temperature of  $\text{SO}_2$  gas and moisture upon the oxidized copper minerals. This bright red crystalline precipitate possesses this property of floating to a remarkable degree. 50 A qualitative test can readily be made in a test tube by boiling off the  $\text{SO}_2$  from a solution of copper in water and  $\text{SO}_2$ , cooling, adding a drop of oil, and shaking vigorously. The red sulfite is immediately carried to the surface by the bubbles, giving a 55 bright red froth. This test may also be car-

ried out by pouring the precipitate and solution into a large watch glass where the sulfite may be made to float on the surface of the water by a little skilful manipulation 60 of the glass. The precipitate can be made to do this even without the addition of oil, but more readily if a little oil is present.

In applying these facts to the treatment of an ore the copper values are converted to 65 the cupro-cupric sulfite by a suitable method or the particles of copper mineral coated with the cupro-cupric sulfite by any suitable method and then the sulfite precipitate or sulfite coated mineral particles are removed 70 from the gangue by flotation either by forming a froth, as is ordinarily done, or by causing them to float away on the surface film.

In a general way the process of my invention may be carried out as follows: If it is necessary to bring all the copper into solution as is the case with roasted pyrite ores containing copper and some oxidized ores in which the copper minerals are very intimately mixed with the gangue, the treatment may be as follows: The ore ground to required fineness is agitated with a solution of  $\text{SO}_2$  in water until all the copper is brought into solution. The mixture is then 85 heated to boiling and agitated until the excess  $\text{SO}_2$  is driven off and the copper precipitated as the cupro-cupric sulfite. The mixture is then cooled and passed to the flotation machine and the sulfite separated 90 from the gangue in a manner similar to the sulfids in the well known sulfid flotation processes.

If it is necessary to bring only part of the copper into solution, the sulfitizing treatment may be as follows: The ore is agitated with a solution of  $\text{SO}_2$  in water until the desired amount of copper has gone into solution. The excess  $\text{SO}_2$  is then driven off and the dissolved copper precipitated as the 100 cupro-cupric sulfite and the particles of the oxidized copper minerals are coated with the sulfite as shown in the following reaction wherein the expression "CuO" is used as a type radical to indicate the combined form 105 of copper present in the mineral:



The cupro-cupric sulfite thus formed coats the oxidized mineral particles. The smaller 110 the amount of copper dissolved the less  $\text{CuSO}_4$  is formed. The addition of sufficient

of a soluble lime compound will cause all the  $\text{CuSO}_4$  formed to be precipitated as the sulfite when the  $\text{SO}_2$  is boiled off as shown below:



After the removal of the excess  $\text{SO}_2$  the pulp mixture is cooled and passed to the 10 flotation machine as noted above.

It is advantageous to bring as little of the copper into solution as possible where the particles may be separated from the gangue by grinding and may be coated with 15 the sulfite and "floated". In this case the moistened ore is treated at proper temperature with  $\text{SO}_2$  gas for a sufficient time to coat the particles with the sulfite and the excess  $\text{SO}_2$  driven off by heating. The reactions in this case are the same as in the previous one but take place only on the surface 20 of the mineral particles. This operation should be carried out without access of air in order to avoid the formation of  $\text{CuSO}_4$ . After the removal of the excess  $\text{SO}_2$  the ore 25 is passed to the flotation machines as indicated above.

A remarkable difference in the appearance of this froth and that in the sulfid flotation 30 process is that the froth in this case is a bright red. This is also the case with the film in the Macquisten tube where the concentrates floating off are a brilliant red.

Tests upon different copper ores by these 35 methods have given most excellent results. For example: An ore carrying 40% copper as carbonate in a sandstone, after a preliminary treatment of only five minutes and driving off the excess  $\text{SO}_2$ , gave a recovery 40 of 95% and a concentrate carrying 26% copper before cleaning or re-treatment; a complex silicious iron ore carrying 1% copper and some gold and silver, after ten minutes' treatment and boiling, gave an extraction of 85% upon the gold, silver, and copper, in a concentrate carrying 12% copper; a heavy iron sulfid ore carrying 2% copper after roasting and thirty minutes' preliminary treatment and boiling gave an 45 extraction of 90%.

I have also found that the gold and silver values present are caused to float by this treatment of oxidized ores. It is probable that the silver is changed to the sulfid in the 50 boiling operation, especially if the ore contains much iron which would go into solution. No special reason can be assigned for the floating of the gold in this case except that it is probably brightened in the preliminary treatment so as to float readily. It is a fact, however, that some ores which do not yield to flotation of the gold and silver by the ordinary methods have given excellent results by this process.

60      Other methods of converting the copper to

the sulfite or coating the copper minerals with the sulfite may be used, such as treatment with a soluble sulfite like calcium bisulfite, or precipitating the Cu from a sulfate solution by means of calcium bisulfite; but these have not given as good results as the method outlined. As it is obviously impossible in the brief scope of this specification to give a complete description of all the chemical methods and mechanical means 75 by which the copper minerals may be converted to the sulfite or coated with the sulfite in the preliminary treatment, I wish it distinctly understood that I do not desire to be limited by the brief description possible in this specification, but only by the scope and spirit of the claims hereunto appended. Moreover, as all the methods of treating the pulp after the sulfitizing treatment can obviously not be covered in a brief 80 specification, I wish it understood that I desire to be limited here also only by the scope and spirit of the appended claims, as the sulfite precipitate and the coated mineral particles, or in other words the sulfited minerals, may be separated from the gangue by any of the well known froth or film flotation methods by any of the ordinary mechanical appliances successfully used 85 in the old sulfid flotation processes. 90

It will be apparent to all metallurgists that this discovery has a wide field of application. Among these applications the following may be mentioned, namely, the treatment of:

Partly oxidized copper ores. The sulfitizing treatment of these ores not only causes the oxidized minerals to float, but also cleans the sulfids so that they float more readily.

Oxidized copper ores in sandstone or other 105 non-soluble gangue. These ores yield very readily to this treatment and give a high extraction and a very clean concentrate.

Heavy iron sulfid ores. By roasting these ores they may be handled without difficulty, 110 the  $\text{SO}_2$  from the roast being absorbed in suitable towers and used as the solvent, or sulfitizing agent, and the heat from the roasting operation being used to drive off the excess  $\text{SO}_2$ .

Many of the ores in these different classes which carry the gold and silver in the sulfids are advantageously treated by this process, the sulfids being cleaned and caused to float more readily by the treatment.

Some of these ores carrying gold and silver along with the copper will give good extractions on the gold and silver as well as the copper.

In the claims I have used the term "flotation" to cover all of the well known methods of flotation either by the frothing or film methods. The term flotation has come into such general use and is so well known that it may be and is commonly used in a general 125 130

way to cover any of the processes or methods by which a mineral compound is separated from the gangue by virtue of its particles not being wet by water to the same degree as the gangue, of adhering to bubbles of air, of being wet by oils to a much greater degree than the gangue, etc., which properties make it possible to separate these mineral particles from the gangue by floating them away on the surface film of water or floating away attached to bubbles, or removing in a froth. The "flotative" properties of the sulfids are now well known and the processes which make use of these properties to separate the sulfids are called flotation processes and the act is called "flotation."

It is in the broad general sense whose application is now so generally acknowledged and understood that I use the term "flotation" in the claims. The newly discovered "flotative" properties of the sulfites are similar to those of the sulfids and any method for using these properties to separate this compound from the gangue is flotation.

Having described my discovery and outlined its applications, what I claim and desire to patent is:

1. The process of concentrating ores which comprises separating cupro-cupric sulfite by flotation.

2. The process of concentrating ores which comprises converting copper minerals therein into cupro-cupric sulfite and separating said converted minerals by flotation.

3. The process of concentrating ores which comprises converting copper minerals therein superficially into cupro-cupric sulfite and separating said converted minerals by flotation.

4. The process of treating copper-containing comminuted ores which comprises subjecting said ores to the action of sulfur dioxide in the presence of water, thereby forming copper sulfite, and heating, thereby forming cupro-cupric sulfite.

5. The process of treating copper-containing comminuted ores which comprises agitating said ores with an aqueous solution of sulfurous acid and subsequently heating, thereby expelling sulfur dioxide and forming cupro-cupric sulfite.

6. The process of treating copper-containing comminuted ores which comprises agitating said ores with an aqueous solution of sulfurous acid to effect complete solution of the copper and subsequently heating, thereby expelling sulfur dioxide and forming cupro-cupric sulfite.

7. The process of treating copper-containing ores which comprises subjecting said ores to the action of sulfur dioxide in the presence of water and in the absence of air, thereby avoiding formation of copper sulfate, and subsequently heating, thereby expelling sulfur dioxide and forming cupro-cupric sulfite.

8. The process of treating copper-containing comminuted ores which comprises agitating said ores with an aqueous solution of sulfur dioxide, thereby forming copper sulfite, adding a soluble lime compound and subsequently heating, thereby expelling sulfur dioxide and forming cupro-cupric sulfite.

9. The process of treating copper-containing comminuted ores which comprises subjecting said ores to the action of sulfur dioxide in the presence of water, thereby forming copper sulfite, and heating, thereby forming cupro-cupric sulfite, and separating said cupro-cupric sulfite by flotation.

10. The process of treating copper-containing comminuted ores which comprises agitating said ores with an aqueous solution of sulfurous acid and subsequently heating, thereby expelling sulfur dioxide and forming cupro-cupric sulfite, and separating said cupro-cupric sulfite by flotation.

11. The process of treating copper-containing comminuted ores which comprises agitating said ores with an aqueous solution of sulfurous acid to effect complete solution of the copper and subsequently heating, thereby expelling sulfur dioxide and forming cupro-cupric sulfite, and separating said cupro-cupric sulfite by flotation.

12. The process of treating copper-containing ores which comprises subjecting said ores to the action of sulfur dioxide in the presence of water and in the absence of air, thereby avoiding formation of copper sulfate, and subsequently heating, thereby expelling sulfur dioxide and forming cupro-cupric sulfite, and separating said cupro-cupric sulfite by flotation.

13. The process of treating copper-containing comminuted ores which comprises agitating said ores with an aqueous solution of sulfur dioxide, thereby forming copper sulfite, adding a soluble lime compound and subsequently heating, thereby expelling sulfur dioxide and forming cupro-cupric sulfite, and separating said cupro-cupric sulfite by flotation.

In testimony whereof I have signed my name to this specification.

NIELS C. CHRISTENSEN.